



US005590447A

**United States Patent**

[19]

Goineau

[11] **Patent Number:** **5,590,447**[45] **Date of Patent:** **Jan. 7, 1997**

[54] **CONTINUOUS PROCESS FROM  
INTERLACING TO WARPING TO PROVIDE  
A HEATHER YARN**

4,644,622 2/1987 Bauer et al. .... 28/172.1  
4,813,161 3/1989 Lesley .  
4,905,355 3/1990 Bauer et al. .  
5,148,586 9/1992 Coons, III ..... 28/271  
5,295,287 3/1994 Chateau .

[75] Inventor: **André M. Goineau**, Spartanburg, S.C.

[73] Assignee: **Milliken Research Corporation**,  
Spartanburg, S.C.

**FOREIGN PATENT DOCUMENTS**

50-26661 9/1975 Japan ..... 28/271  
62-149932 7/1987 Japan ..... 28/172.1

[21] Appl. No.: **540,156**

[22] Filed: **Oct. 6, 1995**

[51] Int. Cl.<sup>6</sup> ..... **D02G 1/18; D02G 1/16;**  
**D02J 1/08**

[52] U.S. Cl. ..... **28/172.1; 28/178; 28/271**

[58] Field of Search ..... 28/172.1, 178,  
28/271

[56] **References Cited**

**U.S. PATENT DOCUMENTS**

3,591,955 7/1971 Fujita ..... 28/271

Primary Examiner—Andy Falik

Attorney, Agent, or Firm—Terry T. Moyer; Earle R. Marden

[57] **ABSTRACT**

Method to continuously merge two multifilament yarns supplied from bobbins on a creel by merging and entangling the two yarns in a commingling air jet and supplying directly to a warper to form a warp beam. The method includes feed rolls upstream and downstream of the air jets providing an overfeed of the yarns to the jet of about 2.3%.

**7 Claims, 1 Drawing Sheet**





FIG. -1-



FIG. -2-

**CONTINUOUS PROCESS FROM  
INTERLACING TO WARPING TO PROVIDE  
A HEATHER YARN**

This invention relates generally to the continuous production of a warp beam of a multiplicity of merged or entangled yarns from a plurality of bobbins mounted in a creel.

It is known to air entangle a multiplicity of yarns from a bobbin into a single yarn and then take up the merged or entangled on another bobbin which is combined with other bobbins and supplied to a warp beam. The supplied yarns can be yarns of the same color or texture or can be yarns of different colors. These yarns normally are taken up on a bobbin prior to warping and require the additional step or steps of loading them onto a creel and then threading them up to a warper to provide a warp beam of such yarns.

It is therefore an object of this invention to provide a continuous process of merging a plurality of yarns from bobbins mounted on a creel and, in line, continuously directing the merged yarns on a warp beam.

Other objects and advantages of the invention will become clearly apparent as the specification proceeds to describe the invention with reference to the accompanying drawing, in which:

FIG. 1 is a side schematic view of the new and improved process and FIG. 2 is a top view taken on line 2—2 of FIG. 1.

Looking now to the drawings, the reference numbers 10 and 12 represent a false twisted single ply, 250 denier, 100 filament polyester yarns that are being supplied from bobbins 13 on a creel 14. In the preferred form of the invention, the yarn 10 is light grey and the yarn 12 is a dark grey in order to form a heather yarn 18 but it should be understood that other synthetic filament yarns, such as nylon, of different deniers, numbers of filaments and colors can be used within the scope of the invention.

The yarns 10 and 12 are delivered from the creel 14 to feed rolls 20 and 21 through a comb 22 which supplies one yarn 10 and one yarn 12 to each air entanglement jet 24 mounted on the air manifold 26 supplying air to each air jet 24 so that they operate at a pressure between 30–90 psi, preferably 60 psi, to entangle each pair of yarns 10 and 12. Since the yarns 10 and 12 are different colors, the entangled yarn 18 has a heather appearance and is basically a two ply, 250 denier, 200 filament yarn. To allow the jets 24 to provide this heather effect, the output feed rolls 30 and 32 are supplying yarn to the warper 34 at a rate of 400 meters/minute which the input feed rolls are supplying yarn at a rate

of about 409 meters providing an overfeed of yarn of about 2.3%. This overfeed can vary between 1 and 4%. Prior to the output rolls 30 and 32 the entangled yarns 18 each pass through a separate space in the dent 36 to maintain them separate as the feed rolls 30 and 32 feed them to the warp beam 38 of the warper 34.

The above described process provides an entangled yarn, preferably a heather yarn, warped and ready for use in a single continuous process from bobbins to the warp beam eliminating the intermediate steps of winding bobbins and recreeling at the warper to form a warp beam. Furthermore, the continuous system described provides a yarn having a heather hand and appearance especially when knit or woven into a fabric.

It is contemplated that modifications of the process can be made without departing from the scope or spirit of the invention and it is desired to be limited only by the scope of the claims.

I claim:

1. A method to continuously produce a warp beam of merged multifilament yarn from at least two false twisted textured yarns wound on individual bobbins having multifilament synthetic yarn thereon, comprising the steps of supplying at least two yarns from separate bobbins to a set of feed rolls, driving said set of feed rolls at a first rate to supply the two yarns to a commingling air jet, commingling the two yarns in the air jet to provide a merged, commingled yarn, providing a second set of feed rolls downstream of the air jet, driving the second set of feed rolls at a rate lower than that of the first set of feed rolls so that the yarns are supplied to the air jet at an overfeed of between 1 to 4%, supplying the commingled yarn from the second set of feed rolls to a warper and forcing a warp beam of commingled yarn on the warp beam.

2. The method of claim 1 wherein the air jet is supplied air at a pressure of about 60 psi.

3. The method of claim 2 wherein the yarn overfeed is about 2.3%.

4. The method of claim 1 wherein the yarn overfeed is about 2.3%.

5. The method of claim 1 wherein the two yarns supplied are of different colors and the commingled yarn is a heather yarn.

6. The method of claim 5 wherein the air jet is supplied air at a pressure of about 60 psi.

7. The method of claim 6 wherein the yarn overfeed is about 2.3%.

\* \* \* \* \*